

July 17, 1951

J. B. LEUZARDER ET AL

2,561,061

GLASS-TO-METAL SEAL AND PROCESS FOR MAKING THE SEAL

Filed Dec. 17, 1947

Fig. 1.



Fig. 2.



Fig. 3.



Fig. 4.



INVENTORS  
J. B. LEUZARDER  
J. PAKJER  
W. J. KNOCHEL

999 nee how  
ATTORNEY

## UNITED STATES PATENT OFFICE

2,561,061

GLASS-TO-METAL SEAL AND PROCESS FOR  
MAKING THE SEAL

John B. Leuzarder, Verona, Jens J. Aakjer, Roselle, and William John Knochel, East Orange, N. J., assignors to Westinghouse Electric Corporation, East Pittsburgh, Pa., a corporation of Pennsylvania

Application December 17, 1947, Serial No. 792,268

6 Claims. (Cl. 49—78)

1

This invention relates to seal and lead-in construction and method of manufacture, and specifically refers to the means and method of sealing lead-in wires or posts through glass enclosures in electrical apparatus such as lamps, electronic tubes and the like.

A commonly used sealing method of the prior art follows the procedure of first beading a lead-in wire with a bead of glass and thereafter sealing the bead to the stem or other glass part of the envelope. This method has required the bead to be twice heated, with cooling taking place during the intervening interval, and also requires double handling, with attendant breakage and contamination, and produces irregular seals, especially as to durability, since each lead-in wire oxidizes during whatever time transpires while exposed and the heat applied. Insufficient oxidation results in poor adhesion of the glass bead to the lead-in wire and excessive oxidation results in formation of leakage paths through the oxide when the envelope is evacuated.

The present invention proposes uniform oxidation of the lead-in wires under controlled conditions and sealing of the bead thereto without material change in the amount of oxide at the seal.

The invention further contemplates stem assembly in a single heating operation for the glass-to-metal and glass-to-glass seals.

A further object of the invention is to both reduce time and steps in fabrication of stem assemblies.

Other objects of the invention will appear to those skilled in the art to which it appertains as the description thereof proceeds, both by direct recitation thereof and by implication from the context.

Referring to the accompanying drawing in which like numerals of reference indicate similar parts throughout the several views;

Figure 1 is an elevation of an electrical device wherein our invention is employed in fabrication of the stem assembly shown therein;

Figure 2 is an elevation, partially broken away, showing the completed stem assembly;

Figure 3 is a sectional view of the stem assembly in process of fabrication and showing portions of the apparatus utilized in carrying out the method involved; and

Figure 4 is a cross-section on line IV—IV of Figure 3.

In the specific embodiment of the invention illustrated in said drawing, the selected electrical device in which the invention is incorporated is

2

an electronic tube of the diode type known specifically as a Rectigon or rectifier, and comprises a vacuum-tight envelope 10, usually of glass, having a screw-base 11 at one end making electrical connection with lead-in wires 12, 13 within the tube which carry therebetween a cathode 14 which is also within the envelope. At the other end of the envelope is a stem assembly 15 which provides a flare 16 the rim of which is integrally sealed to the wall of the envelope at a neck end 17 thereof. The stem assembly includes a lead-in wire or post 18 longitudinally therethrough with a tear-drop glass seal thereon at the inner end of the flare. A press-seal may be employed, however, in place of a tear-drop seal if desired. Within the envelope, the lead-in wire carries an electrode, such as anode 19, in proper spaced relation to above-mentioned cathode 14.

The present invention inheres more particularly in the stem assembly and its method of manufacture. In carrying out the invention, a quantity of lead-in wires are first oxidized according to a fixed schedule so as to have an oxide coating thereon of predetermined character and thickness. Usually the lead-in wires 18 are tungsten and according to this invention are oxidized in groups of one to five hundred at a time. A baking period of five to ten minutes in air at a temperature of approximately 600° C., obtaining an oxide coating from .00003 to .00009 inch, has proved to be the desired range, with preference given to seven and a half minutes baking for a coating of substantially .00006 inch. The lead-in wires 18 are of adequate dimension, say about  $\frac{1}{16}$  inches in diameter, to be sufficiently rigid that they are adapted to serve each as a supporting post for the anode shown herein or for other uses to which adapted.

Fabrication of the stem assembly utilizes power-driven apparatus, of which the portion herein shown includes a rotating sealing head 20 the axis of rotation of which is vertical. Said sealing head 20 is operatively mounted upon and constantly rotated by a usual construction of sealing machine well known in the prior art. The sealing head 20 is hollow and receives a socket member 21 therein to rotate therewith, said socket member having a coaxial socket 22 therein of proper diameter and depth to receive and support the lead-in wire or post 18 coaxial to the axis of rotation and with predetermined protrusion of the post from the upper end of the said member. The seal of the glass portion of the stem is accomplished upon the oxidized post immediately above and where protruding from the member.

Above the socket member 21 as a part of said sealing machine, there is provided a flare support 23 recessed coaxial to the axis of the said member and in spaced relation thereabove, which enables a glass stem-tube 24 to be hung therein by its flare 16 coaxially around the protruding part of the post 18, but with the lower end of the said tube out of contact from said member thereby providing a gap 25 between the lower end of the glass tube and the upper end of the socket member. The flare support 23 rotates at the same speed as and with the rotating sealing head 20 and socket member 21.

Further above the sealing head 20 and above the said flare support 23, also as part of said sealing machine, are provided means for gripping the upper end portion of the post, said means being herein indicated as gripping fingers 26 diametrically opposed to each other on opposite sides of the post. These gripping fingers 26 likewise revolve about the common axis of rotation of the sealing head 20, flare support 23, and post 18, at the same speed as and with the rotating sealing head 20.

In the assembly of the work in the machine, the post 18 is dropped into the socket 22 of the socket member 21 and its upper end is gripped by said gripping fingers 26 for rotating said post; the flared glass stem-tube 24 is hung in the recess of the flare support 23; and a short sleeve of glass herein designated a floating bead 27, which slidably fits upon the protruding portion of the post, is slid down that post until the lower end of said sleeve of glass or floating bead 27 rests upon the upper end of the socket member 21. This bead 27, because of frictional contact, will rotate with the post 18 and socket member 21. The glass preferred for said glass sleeve or floating bead 27 is one of appropriate character to have approximately the same coefficient of expansion as the metal comprising post 18. The glass of flared tube 24 may be of the same characteristic as that of the sleeve, or may be somewhat different in its coefficient of expansion to provide a graded seal from the post 18 to envelope 10.

With the work pieces assembled in the machine as above described, they are simultaneously rotated and flames 28 from burners 29 are played upon the glass tube 24 at the lower end thereof below the flare support 23 and immediately above the socket member 21. Part of the flame and heat enters gap 25 and as a consequence the glass of both the tube 24 and sleeve or bead 27 softens and shrinks inwardly initially at the lower extremity of each. Continued application of the flame results in the tube 24 sealing with sleeve or bead 27 and the bead with the post 18 as a simultaneous or continuing operation of thermal sealing. If so desired, and particularly when sealing more than one lead-in wire in the stem, mechanical pressure may be applied at the side of the tube 24 through which the several wires extend, to press the glass of the tube into sealing unification with the several sleeves or beads 27, thereby forming a flat press at the end of the stem.

It is now appropriate and important to point out that an effective seal between glass and metal in general requires surface oxidation of the metal. In particular, to obtain a vacuum tight seal between glass and tungsten, the surface of the tungsten must be coated with an oxide. The best oxide for tungsten-to-glass seal is tungsten oxide. However, it has been further

determined that excessive oxidation creates a condition of a crust of oxide interposed between the tungsten and the glass, and that such a crust contains shrinkage cracks or crevices through which air may seep longitudinally of the seal and thus void the desired vacuum within the envelope. On the other hand, an oxide coating of minute thickness seems to intermingle with the glass for improving the bond, with the glass actually in engagement with the tungsten, and therefore no crust and no crevices are present. The above described oxidation schedule has been found to give the requisite oxide coating, neither too thin nor too thick.

After the desired oxide coating is applied according to the prescribed schedule, it is important that no further oxidation be instigated during the sealing operation. The high heat employed with flames 28 during sealing promotes oxidation of tungsten. By the present invention, however, lack of oxygen at the seal prevents further oxidation of the tungsten thereat. Lack of oxygen results from (1) the fact that the glass sleeve or bead 27 has sliding fit with the post, (2) from the fact the lower end of the bead rests upon the socket member preventing entry of additional air, (3) from the fact the glass seals first next the lower end of the bead, thereby preventing entry of oxygen from below, and (4) from the fact rising heat and gases in the slight space between post and bead prevent influx of oxygen at the upper end of the bead. Consequently the bead not only constitutes a sealing medium with the tungsten, but during the sealing thereof to the tungsten constitutes a protector against further oxidation of the tungsten within the sealing region. The seal thus effected is one wherein a predetermined amount of the tungsten oxide is presented to and absorbed by the glass juxtaposed to the tungsten bead, so that the mingling of oxide with the glass is confined to practically only the surface layer of the glass next the tungsten thereby strengthening the bond between the glass and tungsten without spreading into and weakening the body of glass by dispersion therein beyond the surface thickness thereof. Penetration of the oxide into the glass, or what is herein termed surface thickness of the glass, appears to be approximately double the thickness of the oxide coating on the metal at the time the seal is effected, that is to say up to about .0002 inch.

We claim:

55. 1. A glass-to-metal seal comprising a metallic part and a glass part thermally bonded, the juxtaposed surface of the glass to the metal having a predetermined quantitatively limited metal oxide therein confined to immediate vicinity of the glass to the metal and providing a surface of intermingled oxide and glass toward and in bonded contact with the metal of said metallic part substantially to the exclusion of oxide film between the glass and metal.

60. 2. A glass-to-metal seal comprising a tungsten part and a glass part thermally bonded, the juxtaposed surface of the glass to the tungsten having a predetermined quantitatively limited metal oxide therein confined to immediate vicinity of the glass to the tungsten and providing a surface of intermingled metal oxide and glass toward and in bonded contact with the tungsten of said tungsten part substantially to the exclusion of metal oxide film between the glass and tungsten parts.

3. A glass-to-metal seal comprising a tungsten part and a glass part thermally bonded, the juxtaposed surface of the glass to the tungsten having a tungsten oxide therein quantitatively limited to an amount of tungsten oxide obtainable from a film thickness on the metal part less than .00009 of an inch and confined to the immediate vicinity of the glass to the tungsten and providing a surface of intermingled tungsten oxide and glass toward and in direct bonded contact with the tungsten of said tungsten part substantially to the exclusion of oxide film between said tungsten part and glass part.

4. A method of effecting a glass-to-metal seal comprising oxidizing a metal part with an oxide coating substantially between .00003 and .00009 inch in thickness, protecting the area to be sealed of the oxidized part and preventing further oxidation thereat, and thermally sealing the glass at the protected part of said oxidized metal area and obtaining dispersion of substantially all of the oxide coating at said area from the metal into the glass and confined to surface penetration in the glass of said oxide and obtaining bonded contact directly with the metal of the metal part by the glass containing the metal oxide.

5. A method of effecting a glass-to-metal seal comprising oxidizing a tungsten lead-in post at a predetermined heat of approximately 600° C. for a predetermined time in the approximate range of five to ten minutes and obtaining a coating of tungsten oxide within the range of substantially .00003 to .00009 inch in thickness on said post, protecting the portion of the length of said post from further oxidation at the area where sealing is to be effected, and thermally sealing glass to said post at said protected area and obtaining dispersion of substantially all of the tungsten oxide coating at said area from said tungsten post into the glass and confined to

surface penetration in the glass of said oxide and obtaining bonded contact directly with the tungsten of the tungsten lead-in post by the glass containing the tungsten oxide.

5 6. A method of effecting glass-to-metal seal of a lead-in post in a stem assembly, comprising supporting a lead-in post in a socket member, applying a glass sleeve on said post with an end of said sleeve against said member, locating a stem tube around said sleeve with the end of said tube towards said member spaced therefrom for providing a gap therebetween for entry of flame and heat to the end margin of said sleeve, and directing a flame to said sleeve and tube next said gap and into said gap for progressively sealing the sleeve to the post beginning at the member-engaging end of the sleeve and simultaneously sealing the tube to said sleeve.

JOHN B. LEUZARDER.

JENS J. AAKJER.

WILLIAM JOHN KNOCHEL.

#### REFERENCES CITED

The following references are of record in the file of this patent:

#### UNITED STATES PATENTS

| Number    | Name    | Date          |
|-----------|---------|---------------|
| 1,692,998 | Ruben   | Nov. 27, 1928 |
| 2,010,145 | Eitel   | Aug. 6, 1935  |
| 2,220,742 | Thorson | Nov. 5, 1940  |

#### FOREIGN PATENTS

| Number     | Country       | Date         |
|------------|---------------|--------------|
| 35 194,673 | Great Britain | Nov. 8, 1923 |

#### OTHER REFERENCES

"Procedures in Experimental Physics," (pg. 24), by John Strong et al., pub. by Prentice-Hall Inc., 40 N. Y., 1944.